

# United States Patent

O'Drobinak et al.

[15] 3,640,785

[45] Feb. 8, 1972

[54] **CASTABLE FLUOROCARBON BINDERS  
FOR PROPELLANTS**

[72] Inventors: John D. O'Drobinak; Martin H. Kaufman, both of China Lake, Calif.

[73] Assignee: The United States of America as represented by the Secretary of the Navy

[22] Filed: Aug. 28, 1964

[21] Appl. No.: 394,379

[52] U.S. Cl. .... 149/88, 149/19, 149/93,  
149/109, 260/32.4, 260/33.8 F, 260/86.1 E,  
260/87.3, 260/89.5 H

[51] Int. Cl. .... C06b 3/00

[58] Field of Search .... 260/89.5, 32.4, 33.8 F, 86.1 E,  
260/87.3, 89.5 H; 149/19, 88, 93, 109

[56] **References Cited**

UNITED STATES PATENTS

|           |         |                       |          |
|-----------|---------|-----------------------|----------|
| 2,811,501 | 10/1957 | Stedry.....           | 260/41   |
| 2,839,513 | 6/1958  | Ahlbrecht et al. .... | 260/86.1 |
| 3,022,149 | 2/1962  | Cramer.....           | 149/19   |
| 3,023,573 | 3/1962  | Friedman.....         | 149/19 X |
| 3,235,421 | 2/1966  | Berenbaum et al. .... | 149/19   |
| 3,255,059 | 6/1966  | Hamermesh.....        | 149/19   |

3,493,546 2/1970 Cottrill et al..... 149/19 X

Primary Examiner—Leland A. Sebastian

Attorney—G. J. Rubens, P. H. Firsht and V. C. Muller

**EXEMPLARY CLAIM**

1. A castable binder composition comprising the following constituents:

a fluorocarbon monomer selected from the group consisting of 1H, 1H, 9H-hexadecafluoro-1-monomethacrylate, 1H, 1H, 9H-hexadecafluoro-1-nonanoacrylate, 1H, 1H, 7H-dodecafluoro-1-heptanoacrylate, 1H, 1H, 5H-octafluoro-1-pentanoacrylate and mixtures thereof;

a plasticizer selected from the group consisting of triethylene glycol dinitrate, pentaerythritol trinitrate, trimethylol ethane trinitrate, diethylene glycol dinitrate, butanediol dinitrate, a copolymer of vinylidene fluoride and perfluoropropylene, bis(2-fluoro-2,2-dinitroethyl) formal and mixtures thereof;

a cross-linking agent selected from the group consisting of triallylcyanurate and divinyl benzene; and

a catalyst selected from the group consisting of azobisisobutyronitrile, benzoyl peroxide, dichlorobenzoyl peroxide and methylethylketone peroxide.

**19 Claims, No Drawings**

## CASTABLE FLUOROCARBON BINDERS FOR PROPELLANTS

The invention herein described may be manufactured and used by or for the Government of the United States of America for governmental purposes without the payment of any royalties thereon or therefor.

The present invention relates to new fluorocarbon binder compositions and to the preparation thereof.

A great need has been demonstrated in the fields of propellants, explosives and pyrotechnics for a dense binder which would be processed by casting operations. Work on metallized extruded fluorocarbon propellants has shown that propellants with high boost velocity and moderate to high specific impulses could be obtained using these nonenergetic but high-density binders. In volume limited rocket and missile systems density plays an extremely important role in determining their range. These extruded fluorocarbon propellants have done much to increase their range. The limiting factor of the extruded fluorocarbon propellants has been in obtaining large diameter grains and various shapes. The castable fluorocarbon propellants made possible by the present novel binder system overcome this limiting factor. Extruded fluorocarbon pyrotechnic materials and isostatically pressed fluorocarbon explosives have been demonstrated to be superior to their nonfluorocarbon counterparts. However, the limiting factor of these extruded and pressed materials has been the inability to obtain various odd-shaped materials other than the simple conventional shapes, but with the castable fluorocarbon binder, this limitation factor has been eliminated. The present invention contemplates using a free-radical addition-type polymerization to form a binder which can be used directly in castable propellant, explosive, and pyrotechnic formulations.

It is therefore an object of this invention to provide a new binder for use in various propellant and explosive formulations which will enable casting of the final product into any desired shape.

Another object is to provide a binder which when used for propellant formulations will form a castable product which maintains the ballistic characteristics of extruded propellants.

Still another object is to provide a new binder material which will save time in manufacturing a finished propellant grain.

A further object is to provide a method for preparing a dense binder which will add increased boost velocity to cast propellants.

A still further object is to provide a new material that can be used as a binder with a variety of propellant formulations which can be cast into large-diameter rocket motor grains.

Other objects, advantages and novel features of the invention will become readily apparent from the following detailed description.

The composition of the present invention for castable fluorocarbon binders comprises a fluorocarbon monomer selected from the group consisting of 1H, 1H, 9H-hexadecafluoro-1-monomethacrylate, 1H, 1H, 9H-hexadecafluoro-1-nonanoacrylate, 1H, 1H, 7H-dodecafluoro-1-heptanoacrylate, 1H, 1H, 5H-octafluoro-1-pentanoacrylate and mixtures thereof; a plasticizer selected from the group consisting of triethylene glycol dinitrate, pentaerythritol trinitrate, trimethylol ethane trinitrate, diethylene glycol dinitrate, butanediol dinitrate, a copolymer of vinylidene fluoride and perfluoropropylene (Viton) bis(2-fluoro-2,2-dinitroethyl) formal, a fluorinated polyester and mixtures thereof; a cross-linking agent selected from the group consisting of triallylcyanurate and divinyl benzene; and a catalyst selected from the group consisting of azo-bisisobutyronitrile, benzoyl peroxide, dichlorobenzoyl peroxide, and methyl ethyl ketone peroxide.

Vinyl monomers selected from the group consisting of acrylic acid, acrylonitrile, vinylacetate, dinitropropylacrylate and styrene have also been admixed with the fluorocarbon monomers used above and the resulting binder compositions tested successfully, as shown herein. The polymerized

fluorinated monomers such as Viton and fluorinated polyester influence the viscosity of the binder composition thereby permitting efficient loading of solid fuel and oxidizer ingredients of the various propellant formulations utilizing the present binder formulations.

The cross-linking agents apparently form a three-dimensional polymeric network with the fluorocarbon monomers which provide improved physical properties at the elevated temperatures at which the binder composition is to be used.

10 Certain wetting agents may be added as processing aids in the manufacture of the present formulation. Among those found suitable were perfluorooctanoic acid and phosphoric acid esters of fluoroalcohols.

15 The following are representative examples of the successful combinations utilizing a free-radical addition-type polymerization. These examples should not be considered as limiting the invention. They have been divided into groups according to test data results on elongation and density and abbreviations identified hereinafter have been used for the compounds used in the formulations.

20 Identification of the abbreviations referred to above are as follows:

|    |                   |                                                                                                                                       |
|----|-------------------|---------------------------------------------------------------------------------------------------------------------------------------|
| 25 | TEGDN             | Triethylene glycol dinitrate                                                                                                          |
|    | PETRIN            | Pentaerythritol trinitrate                                                                                                            |
|    | TMETN             | Trimethylol ethane trinitrate                                                                                                         |
|    | DEGDN             | Diethylene glycol dinitrate                                                                                                           |
|    | BDDN              | 1,4-butanediol dinitrate                                                                                                              |
|    | FEFO              | Bis(2-fluoro-2,2-dinitroethyl) formal                                                                                                 |
|    | V—Viton           | (copolymer of vinylidene fluoride and perfluoropropylene)                                                                             |
| 30 | PE                | Polyester                                                                                                                             |
|    | FPE               | Fluorinated polyester                                                                                                                 |
|    | C <sub>8</sub> MA | 1H, 1H, 9H-hexadecafluoro-1-nanomethacrylate                                                                                          |
|    | C <sub>9</sub> A  | 1H, 1H, 9H-hexadecafluoro-1-nonanoacrylate                                                                                            |
|    | C <sub>10</sub> A | 1H, 1H, 7H-dodecafluoro-1-heptanoacrylate                                                                                             |
|    | AA                | 1H, 1H, 5H-octafluoro-1-pentanoacrylate                                                                                               |
|    | AN                | Acrylic acid                                                                                                                          |
|    | VA                | Acrylonitrile                                                                                                                         |
|    | St                | Vinylacetate                                                                                                                          |
|    | DNPA              | Styrene                                                                                                                               |
|    | TAC               | Dinitropropylacrylate                                                                                                                 |
|    | DVB               | Triallylcyanurate                                                                                                                     |
|    | Cat.              | Divinyl benzene                                                                                                                       |
|    |                   | Catalyst — free-radical examples, azo-bis-iso-butyronitrile, benzoyl peroxide, dichlorobenzoyl peroxide, methyl ethyl ketone peroxide |

### EXAMPLE I

| Sample | Elongation—0 to 300% |                  |     | % by weight |
|--------|----------------------|------------------|-----|-------------|
|        | C <sub>8</sub> MA    | C <sub>9</sub> A | St. |             |
| 55     |                      |                  |     |             |
| No.    |                      |                  |     |             |
| 1      | 99                   |                  |     | 1           |
| 2      | 89                   |                  | 10  | 1           |
| 3      | 79                   |                  | 20  | 1           |
| 4      | 69                   |                  | 30  | 1           |
| 5      | 59                   |                  | 40  | 1           |
| 6      | 49                   |                  | 50  | 1           |

### EXAMPLE II

| Sample No.               | Elongations—from about 100 to 300% |                  |     |       |
|--------------------------|------------------------------------|------------------|-----|-------|
|                          | C <sub>8</sub> MA                  | C <sub>9</sub> A | St. | TAC   |
| 65                       |                                    |                  |     |       |
| Desnity—1.50-1.80 g./cc. |                                    |                  |     |       |
|                          | Composition—% by weight            |                  |     |       |
|                          | C <sub>9</sub> A                   | St.              | TAC | Cat.* |
| 1                        | 79                                 | 19.5             |     | 1.0   |
| 2                        | 80                                 | 19.6             |     | 0.3   |
| 3                        | 80                                 | 14.6             | 5.0 | 0.3   |
| 4                        | 78                                 | 16.6             | 5.0 | 0.3   |
| 5                        | 75                                 | 19.6             | 5.0 | 0.3   |
| 6                        |                                    | 95.75            |     | 4.0   |
|                          |                                    |                  |     | 0.25  |

3,640,785

3

|   |       |     |      |
|---|-------|-----|------|
| 7 | 96.75 | 3.0 | 0.25 |
| 8 | 97.75 | 2.0 | 0.25 |
| 9 | 98.75 | 1.0 | 0.25 |

4

## EXAMPLE VII

Elongation—about 200 to 400%  
Density—1.5-1.80

\*Azo-bisisobutyronitrile

## EXAMPLE III

Elongations—from about 250 to 300%

Densities—1.5-1.8g./cc.

Composition, percent by weight

| Sample No. | C <sub>9</sub> MA | C <sub>5</sub> A | AA  | AN  | VA | TAC | Cat. | 10  |
|------------|-------------------|------------------|-----|-----|----|-----|------|-----|
| 1          | 79                | 15               | 5   |     |    |     |      | 1   |
| 2          | 79                | 15               |     | 5   |    |     |      | 1   |
| 3          | 79                | 17               | 3   |     |    |     |      | 1   |
| 4          | 79                | 16               | 3   |     |    | 1   |      | 1   |
| 5          | 79                | 17               |     | 3   |    |     |      | 1   |
| 6          | 79                | 15               |     |     | 5  |     |      | 1   |
| 7          | 79                | 17               | 1.5 | 1.5 |    |     |      | 1   |
| 8          | 79                | 17.5             | 1.5 | 1.5 |    |     |      | 0.5 |
| 9          | 79                | 17.7             | 1.5 | 1.5 |    |     |      | 0.3 |
| 10         | 80                | 18               | 1   |     |    |     |      | 1   |
| 11         | 80                | 18               | 1.5 |     |    |     |      | 0.5 |
| 12         | 79                | 19.5             |     |     |    | 1   | 0.5  |     |

## EXAMPLE IV

Elongations—0 to 200%

Density—1.50-1.80 g./cc.

| Sample No. | Composition—% by weight |                  |                  |      | Cat. |
|------------|-------------------------|------------------|------------------|------|------|
|            | C <sub>9</sub> MA       | C <sub>5</sub> A | C <sub>7</sub> A | TAC  |      |
| 1          | 79.9                    |                  | 20.0             |      | 0.1  |
| 2          |                         | 59.9             | 40.0             |      | 0.1  |
| 3          |                         |                  | 98.9             | 1.0  | 0.1  |
| 4          |                         |                  | 99.7             | 0.2  | 0.1  |
| 5          |                         |                  | 59.9             | 39.8 | 0.3  |
| 6          |                         |                  | 70.0             | 29.6 | 0.3  |
| 7          |                         |                  | 80.0             | 19.6 | 0.3  |

## EXAMPLE V

Elongations—about 250%

Densities—1.50-1.80 g./cc.

| Sample No. | Composition, percent by weight |                  |     |     |     | Cat. |
|------------|--------------------------------|------------------|-----|-----|-----|------|
|            | C <sub>9</sub> A               | C <sub>5</sub> A | AN  | AA  | TAC |      |
| 1          | 65                             | 29.6             | 5.0 |     | 0.3 | 0.1  |
| 2          | 70                             | 29.6             |     | 0.3 | 0.1 |      |
| 3          | 66                             | 29.6             | 4.0 |     | 0.3 | 0.1  |
| 4          | 67                             | 29.6             | 3.0 |     | 0.3 | 0.1  |
| 5          | 68                             | 29.6             | 2.0 |     | 0.3 | 0.1  |
| 6          | 78                             | 16.6             | 5.0 |     | 0.3 | 0.1  |
| 7          | 80                             | 19.6             |     | 0.3 | 0.1 |      |
| 8          | 85                             | 14.6             |     | 0.3 | 0.1 |      |
| 9          | 65                             | 29.6             |     | 5.0 | 0.3 | 0.1  |
| 10         | 66                             | 29.6             |     | 4.0 | 0.3 | 0.1  |
| 11         | 67                             | 29.6             |     | 3.0 | 0.3 | 0.1  |

35

## EXAMPLE IX

Elongation—about 400%  
Densities—1.5-1.80 g./cc.

| Sample No. | composition—% by weight |                  |      |     | Cat. |
|------------|-------------------------|------------------|------|-----|------|
|            | C <sub>9</sub> A        | C <sub>7</sub> A | V    | St  |      |
| 1          | 65                      | 21.9             | 13.0 |     | 0.1  |
| 2          | 75                      | 11.9             | 13.0 |     | 0.1  |
| 3          | 86.9                    |                  | 13.0 |     | 0.1  |
| 4          | 58                      | 29.9             | 12.0 |     | 0.1  |
| 5          | 55                      | 27.9             | 12.0 | 5.0 | 0.1  |

50

## EXAMPLE VI

Elongation—about 250%

Densities—1.5-1.80 g./cc.

| Sample No. | Composition—% by weight |                  |     |     | Cat. |
|------------|-------------------------|------------------|-----|-----|------|
|            | C <sub>9</sub> A        | C <sub>5</sub> A | St. | TAC |      |
| 1          | 65                      | 29.6             | 5.0 | 0.3 | 0.1  |
| 2          | 65                      | 29.3             | 5.0 | 0.6 | 0.1  |
| 3          | 65                      | 29               | 5.0 | 0.9 | 0.1  |

Elongation—about 400%

Densities—1.5-1.8 g./cc.

Composition, percent by weight

| Sample No. | C <sub>9</sub> A | C <sub>7</sub> A | V    | St  | TMETN | PETRIN | Cat. |
|------------|------------------|------------------|------|-----|-------|--------|------|
| 1          | 53               | 24.9             | 12.0 | 5.0 |       | 5.0    | 0.1  |
| 2          | 53               | 24.9             | 12.0 | 5.0 |       | 5.0    | 0.1  |

60

Elongation—about 150 to 350%  
Densities—1.5-1.8 g./cc.

Composition, percent by weight

| Sample No. | C <sub>9</sub> MA | C <sub>5</sub> A | V  | PE | FPE | FEFO | DNPA | Cat. | TAC |
|------------|-------------------|------------------|----|----|-----|------|------|------|-----|
| 1          | 63                | 21.8             | 13 | 2  |     |      |      | 0.2  |     |
| 2          | 61                | 20.8             | 13 | 5  |     |      |      | 0.2  |     |
| 3          | 58                | 17.7             | 12 |    |     | 15   |      | 0.3  |     |
| 4          | 50                | 12.7             | 12 |    |     | 20   |      | 0.3  |     |
| 5          | 64                | 20.8             |    |    | 15  |      |      | 0.2  |     |
| 6          | 61                | 18.8             |    |    | 20  |      |      | 0.2  |     |
| 7          | 60                | 24.7             |    |    |     |      | 15   | 0.3  |     |
| 8          | 55                | 24.7             |    |    |     |      | 20   | 0.3  |     |
| 9          | 63.4              | 20.5             | 10 |    |     |      | 5    | 0.1  | 1   |
| 10         | 58.4              | 20.5             | 10 |    |     |      | 10   | 0.1  | 1   |
| 11         | 53.4              | 20.5             | 10 |    |     |      | 15   | 0.1  | 1   |

EXAMPLE XI

## EXAMPLE XII

Elongation—about 250%  
Densities—1.50-1.80 g./cc.

| Sample No. | Composition, percent by weight |                  |    |     |      |       |       |       |
|------------|--------------------------------|------------------|----|-----|------|-------|-------|-------|
|            | C <sub>9</sub> MA              | C <sub>8</sub> A | V  | TAC | Cat. | TMETN | DEGDN | BDDN  |
| 1          | 61.7                           | 22.25            | 10 | 1   | 0.05 | 5     | ----- | ----- |
| 2          | 56.7                           | 22.25            | 10 | 1   | 0.05 | 10    | ----- | ----- |
| 3          | 51.7                           | 22.25            | 10 | 1   | 0.05 | 15    | ----- | ----- |
| 4          | 46.7                           | 22.15            | 10 | 1   | 0.05 | 20    | ----- | ----- |
| 5          | 61.7                           | 22.25            | 10 | 1   | 0.05 | 5     | ----- | ----- |
| 6          | 56.7                           | 22.25            | 10 | 1   | 0.05 | 10    | ----- | ----- |
| 7          | 51.7                           | 22.25            | 10 | 1   | 0.05 | 15    | ----- | ----- |
| 8          | 46.7                           | 22.25            | 10 | 1   | 0.05 | 20    | ----- | ----- |
| 9          | 61.7                           | 22.25            | 10 | 1   | 0.05 | ----- | 10    | ----- |
| 10         | 56.7                           | 22.25            | 10 | 1   | 0.05 | ----- | 15    | ----- |
| 11         | 51.7                           | 22.25            | 10 | 1   | 0.05 | ----- | 20    | ----- |
| 12         | 46.7                           | 22.25            | 10 | 1   | 0.05 | ----- | 20    | ----- |

## EXAMPLE XIII

Elongation—above 250%  
Densities—1.50-1.80 g./cc.

| Sample No. | Composition, percent by weight |                  |    |     |      |        |       |       |       |       |
|------------|--------------------------------|------------------|----|-----|------|--------|-------|-------|-------|-------|
|            | C <sub>9</sub> MA              | C <sub>8</sub> A | V  | TAC | Cat. | PETRIN | TEGDN | BDDN  | DEGDN | TMETN |
| 1          | 56                             | 21.9             | 10 | 2   | 0.1  | 10     | ----- | ----- | ----- | ----- |
| 2          | 51                             | 21.9             | 10 | 2   | 0.1  | 15     | ----- | ----- | ----- | ----- |
| 3          | 56                             | 21.9             | 10 | 2   | 0.1  | -----  | 10    | ----- | ----- | ----- |
| 4          | 51                             | 21.9             | 10 | 2   | 0.1  | -----  | 15    | ----- | ----- | ----- |
| 5          | 56                             | 21.9             | 10 | 2   | 0.1  | -----  | 10    | ----- | ----- | ----- |
| 6          | 51                             | 21.9             | 10 | 2   | 0.1  | -----  | 15    | ----- | ----- | ----- |
| 7          | 56                             | 21.9             | 10 | 2   | 0.1  | -----  | 10    | ----- | ----- | ----- |
| 8          | 51                             | 21.9             | 10 | 2   | 0.1  | -----  | 15    | ----- | ----- | ----- |
| 9          | 56                             | 21.9             | 10 | 2   | 0.1  | -----  | 10    | ----- | ----- | ----- |
| 10         | 51                             | 21.9             | 10 | 2   | 0.1  | -----  | 15    | ----- | ----- | ----- |

## EXAMPLE XIV

Elongation—about 200%  
Densities—1.5-1.80 g./cc.

| Sample No. | Composition, percent by weight |                  |    |      |     |       |        |
|------------|--------------------------------|------------------|----|------|-----|-------|--------|
|            | C <sub>9</sub> MA              | C <sub>8</sub> A | V  | Cat. | TAC | TMETN | PETRIN |
| 1          | 59                             | 18.8             | 10 | 0.2  | 2   | 10    | -----  |
| 2          | 56                             | 16.8             | 10 | 0.2  | 2   | 15    | -----  |
| 3          | 59                             | 18.8             | 10 | 0.2  | 2   | ----- | 10     |
| 4          | 56                             | 16.8             | 10 | 0.2  | 2   | ----- | 15     |
| 5          | 56                             | 17.8             | 10 | 0.2  | 1   | 10    | -----  |
| 6          | 56                             | 17.8             | 10 | 0.2  | 1   | ----- | 10     |

## EXAMPLE XV

Elongation—about 250%  
Densities—1.50-1.80 g./cc.

| Sample No. | Composition, percent by weight |                  |    |    |     |      |       |        |       |       |        |
|------------|--------------------------------|------------------|----|----|-----|------|-------|--------|-------|-------|--------|
|            | C <sub>9</sub> MA              | C <sub>8</sub> A | V  | St | TAC | Cat. | DEGDN | TEMETN | BDDN  | TEGDN | PETRIN |
| 1          | 55.9                           | 18               | 10 | 5  | 1   | 0.01 | 10    | -----  | ----- | ----- | -----  |
| 2          | 52.9                           | 16               | 10 | 5  | 1   | 0.1  | 15    | -----  | ----- | ----- | -----  |
| 3          | 55.9                           | 18               | 10 | 5  | 1   | 0.1  | ----- | 10     | ----- | ----- | -----  |
| 4          | 52.9                           | 16               | 10 | 5  | 1   | 0.1  | ----- | 15     | ----- | ----- | -----  |
| 5          | 55.9                           | 18               | 10 | 5  | 1   | 0.1  | ----- | 10     | ----- | ----- | -----  |
| 6          | 52.9                           | 16               | 10 | 5  | 1   | 0.1  | ----- | 15     | ----- | ----- | -----  |
| 7          | 55.9                           | 18               | 10 | 5  | 1   | 0.1  | ----- | 15     | ----- | 10    | -----  |
| 8          | 52.9                           | 16               | 10 | 5  | 1   | 0.1  | ----- | -----  | 10    | ----- | -----  |
| 9          | 55.9                           | 18               | 10 | 5  | 1   | 0.1  | ----- | -----  | 15    | ----- | -----  |
| 10         | 52.9                           | 16               | 10 | 5  | 1   | 0.1  | ----- | -----  | 15    | ----- | -----  |

## EXAMPLE XVI

Elongation—about 200%  
Densities—1.50-1.80 g./cc.

| Sample No. | Composition, percent by weight |                  |    |    |     |      |       |       |       |       |        |
|------------|--------------------------------|------------------|----|----|-----|------|-------|-------|-------|-------|--------|
|            | C <sub>9</sub> MA              | C <sub>8</sub> A | V  | St | TAC | Cat. | BDDN  | DEGDN | TMETN | TEGDN | PETRIN |
| 1          | 54.9                           | 18               | 10 | 5  | 2   | 0.1  | 10    | ----- | ----- | ----- | -----  |
| 2          | 52.9                           | 15               | 10 | 5  | 2   | 0.1  | 15    | ----- | ----- | ----- | -----  |
| 3          | 54.9                           | 18               | 10 | 5  | 2   | 0.1  | ----- | 10    | ----- | ----- | -----  |
| 4          | 52.9                           | 15               | 10 | 5  | 2   | 0.1  | ----- | 15    | ----- | ----- | -----  |
| 5          | 54.9                           | 18               | 10 | 5  | 2   | 0.1  | ----- | 15    | ----- | 10    | -----  |
| 6          | 52.9                           | 15               | 10 | 5  | 2   | 0.1  | ----- | ----- | 10    | ----- | -----  |
| 7          | 54.9                           | 18               | 10 | 5  | 2   | 0.1  | ----- | ----- | 15    | ----- | -----  |
| 8          | 52.9                           | 15               | 10 | 5  | 2   | 0.1  | ----- | ----- | 10    | ----- | -----  |
| 9          | 54.9                           | 18               | 10 | 5  | 2   | 0.1  | ----- | ----- | 15    | ----- | -----  |
| 10         | 52.9                           | 15               | 10 | 5  | 2   | 0.1  | ----- | ----- | 15    | ----- | -----  |

The above formulations may be mixed in three ways to control the viscosity:

a. The fluorinated monomer mixture such as shown in Example I, sample No. 3 is polymerized to about 5 to 20 percent

whereby the viscosity increases to about the consistency of honey;

b. A fluorinated polymeric plasticizer such as Viton can be dissolved in acetone followed by the addition of one of the

fluorinated monomers such as 1,1,5-trihydro-octafluoro-1-pentanoacrylate, with mixing until a homogeneous solution is obtained. The acetone is then removed by evaporation;

c. A fluorinated plasticizer such as Viton can be cut up into small pieces to create a large surface and dissolved in one of the fluorinated monomers with constant mixing and/or heat. A catalyst is dissolved in the cooled solution or in the mixture to which the comonomer previously prepared has been added.

By using the fluorinated monomers instead of acetone the step necessary for removal of the acetone is eliminated. This process may take a little longer to dissolve the Viton.

Obviously many modifications and variations of the present invention are possible in the light of the above teachings. It is therefore to be understood that within the scope of the appended claims the invention may be practiced otherwise than as specifically described.

What is claimed is:

1. A castable binder composition comprising the following constituents:

- a fluorocarbon monomer selected from the group consisting of 1H, 1H, 9H-hexadecafluoro-1-monomethacrylate, 1H, 1H, 9H-hexadecafluoro-1-nonanoacrylate, 1H, 1H, 7H-dodecafluoro-1-heptanoacrylate, 1H, 1H, 5H-octafluoro-1-pentanoacrylate and mixtures thereof;
- a plasticizer selected from the group consisting of triethylene glycol dinitrate, pentaerythritol trinitrate, trimethylol ethane trinitrate, diethylene glycol dinitrate, butanediol dinitrate, a copolymer of vinylidene fluoride and perfluoropropylene, bis(2-fluoro-2,2-dinitroethyl) formal and mixtures thereof;
- a cross-linking agent selected from the group consisting of triallylcyanurate and divinyl benzene; and
- a catalyst selected from the group consisting of azo-bisisobutyronitrile, benzoyl peroxide, dichlorobenzoyl peroxide and methylethylketone peroxide.

2. A castable binder composition comprising the following constituents:

| Constituents                                 | Percent by weight |
|----------------------------------------------|-------------------|
| 1H, 1H, 9H-hexadecafluoro-1-monomethacrylate | 46-62             |
| 1H, 1H, 5H-octafluoro-1-pentanoacrylate      | 16-23             |
| Copolymer of vinylidene fluoropropylene      | 10                |
| Triallylcyanurate                            | 1-2               |
| Azo-bisisobutyronitrile                      | 0.05-0.2          |
| Triethylene glycol trinitrate                | 5-20              |

3. A castable binder composition comprising the following constituents:

| Constituents                                            | Percent by weight |
|---------------------------------------------------------|-------------------|
| 1H, 1H, 9H-hexadecafluoro-1-monomethacrylate            | 46-58             |
| 1H, 1H, 5H-octafluoro-1-pentanoacrylate                 | 21-23             |
| Copolymer of vinylidene fluoride and perfluoropropylene | 10                |
| Triallylcyanurate                                       | 1-2               |
| Azo-bisisobutyronitrile                                 | 0.05-0.1          |
| Diethylene glycol dinitrate                             | 10-20             |

4. A castable binder composition comprising the following constituents:

| Constituents                                            | Percent by weight |
|---------------------------------------------------------|-------------------|
| 1H, 1H, 9H-hexadecafluoro-1-monomethacrylate            | 46-62             |
| 1H, 1H, 5H-octafluoro-1-pentanoacrylate                 | 21-23             |
| Copolymer of vinylidene fluoride and perfluoropropylene | 10                |

|                          |          |
|--------------------------|----------|
| Triallylcyanurate        | 1-2      |
| Benzoyl peroxide         | 0.05-0.1 |
| 1,4-butanediol dinitrate | 5-20     |

5. A castable binder composition comprising the following constituents:

| Constituents                                            | Percent by weight |
|---------------------------------------------------------|-------------------|
| 1H, 1H, 9H-hexadecafluoro-1-monomethacrylate            | 51-56             |
| 1H, 1H, 5H-octafluoro-1-pentanoacrylate                 | 16-22             |
| Copolymer of vinylidene fluoride and perfluoropropylene | 10                |
| Triallylcyanurate                                       | 1-2               |
| Azo-bisisobutyronitrile                                 | 0.05-0.2          |
| Pentaerythritol trinitrate                              | 10-15             |

6. A castable binder composition comprising the following constituents:

|                                                                                                                                                                                                                                                                                                                        |    |
|------------------------------------------------------------------------------------------------------------------------------------------------------------------------------------------------------------------------------------------------------------------------------------------------------------------------|----|
| a fluorocarbon monomer selected from the group consisting of 1H, 1H, 9H-hexadecafluoro-1-monomethacrylate, 1H, 1H, 9H-hexadecafluoro-1-nonanoacrylate, 1H, 1H, 7H-dodecafluoro-1-heptanoacrylate, 1H, 1H, 5H-octafluoro-1-pentaacrylate and mixtures thereof;                                                          | 20 |
| a vinyl monomer selected from the group consisting of acrylic acid, acrylonitrile, vinylacetate, dinitropropylacrylate, styrene and mixtures thereof;                                                                                                                                                                  | 25 |
| a plasticizer selected from the group consisting of triethylene glycol dinitrate, pentaerythritol trinitrate, trimethylol ethane trinitrate, diethylene glycol dinitrate, butanediol dinitrate, a copolymer of vinylidene fluoride and perfluoropropylene, bis(2-fluoro-2,2-dinitroethyl) formal and mixtures thereof; | 30 |
| a cross-linking agent selected from the group consisting of triallylcyanurate and divinyl benzene; and                                                                                                                                                                                                                 | 35 |
| a catalyst selected from the group consisting of azo-bisisobutyronitrile, benzoyl peroxide, dichlorobenzoyl peroxide and methylethylketone peroxide.                                                                                                                                                                   | 40 |

7. A castable binder composition comprising the following constituents:

| Constituents                                            | Percent by weight |
|---------------------------------------------------------|-------------------|
| 1H, 1H, 9H-hexadecafluoro-1-monomethacrylate            | 52-56             |
| 1H, 1H, 5H-octafluoro-1-pentanoacrylate                 | 15-18             |
| Copolymer of vinylidene fluoride and perfluoropropylene | 10                |
| Styrene                                                 | 5                 |
| Triallylcyanurate                                       | 1-2               |
| Benzoyl peroxide                                        | 0.05-0.2          |
| Diethylene glycol dinitrate                             | 10-15             |

8. The composition of claim 7 with trimethylol ethane trinitrate in lieu of diethylene glycol dinitrate.

9. The composition of claim 7 with 1,4-butanediol dinitrate in lieu of diethylene glycol dinitrate.

10. The composition of claim 7 with pentaerythritol trinitrate in lieu of diethylene glycol dinitrate.

11. The composition of claim 7 with triethylene glycol dinitrate in lieu of diethylene glycol dinitrate.

12. A fluorocarbon binder composition comprising the following constituents:

|                                                                                                                                                                                                                                                                 |    |
|-----------------------------------------------------------------------------------------------------------------------------------------------------------------------------------------------------------------------------------------------------------------|----|
| a fluorocarbon monomer selected from the group consisting of 1H, 1H, 9H-hexadecafluoro-1-monomethacrylate, 1H, 1H, 9H-hexadecafluoro-1-nonanoacrylate, 1H, 1H, 7H-dodecafluoro-1-heptanoacrylate, 1H, 1H, 5H-octafluoro-1-pentanoacrylate and mixtures thereof; | 70 |
| a cross-linking agent selected from the group consisting of triallylcyanurate and divinyl benzene; and                                                                                                                                                          | 75 |
| a catalyst selected from the group consisting of azo-bisisobutyronitrile, benzoyl peroxide, dichlorobenzoyl peroxide, and methylethylketone peroxide.                                                                                                           | 75 |

13. A fluorocarbon binder composition comprising the following constituents:

1H, 1H, 9H-hexadecafluoro-1-nonanomethacrylate  
1H, 1H, 5H-octafluoro-1-pentanoacrylate  
Triallycyanurate  
Azo-bisisobutyronitrile.

14. A fluorocarbon binder composition comprising the following constituents:

1H, 1H, 5H-octafluoro-1-pentanoacrylate  
Triallycyanurate  
Azo-bisisobutyronitrile.

15. A fluorocarbon binder composition comprising the following constituents:

| Constituents         | Percent by weight | 15 |
|----------------------|-------------------|----|
| Fluorocarbon monomer | 95-99             |    |
| Cross-linking agent  | 0.3-5             |    |
| Catalyst             | 0.5-1             |    |

20

said fluorocarbon monomer selected from a group consisting of 1H, 1H, 9H-hexadecafluoro-1-nonanoacrylate, 1H, 1H, 7H-dodecafluoro-1-heptanoacrylate, 1H, 1H, 5H-octafluoro-1-pentanoacrylate, 1H, 1H, 9H-hexadecafluoro-1-nonanomethacrylate;

said cross-linking agent selected from a group consisting of triallycyanurate and divinyl benzene; and

said catalyst selected from the group consisting of azo-bisisobutyronitrile, benzoyl peroxide, dichlorobenzoyl peroxide and methylethylketone peroxide.

16. A binder composition comprising the following constituents:

| Constituents         | Percent by weight | 35 |
|----------------------|-------------------|----|
| Fluorocarbon monomer | 94-96             |    |
| Vinyl monomer        | 1-5               |    |
| Cross-linking agent  | 0.3-4             |    |
| Catalyst             | 0.1-1             |    |

40

said fluorocarbon being a member selected from a group consisting of 1H, 1H, 9H-hexadecafluoro-1-monomethacrylate, 1H, 1H, 9H-hexadecafluoro-1-nonanoacrylate, 1H, 1H, 7H-dodecafluoro-1-heptanoacrylate, 1H, 1H, 5H-octafluoro-1-pentanoacrylate and mixtures thereof;

said vinyl monomer being a member selected from a group consisting of acrylic acid, acrylonitrile, vinylacetate, dinitropropylacrylate and styrene;

50

said cross-linking agent being a member selected from the group consisting of triallycyanurate and divinyl benzene; and

said catalyst being a member selected from the group consisting of azo-bisisobutyronitrile, benzoyl peroxide, dichlorobenzoyl peroxide and methylethylketone peroxide.

17. A binder composition comprising the following constituents:

| Constituents                                 | Percent by weight |
|----------------------------------------------|-------------------|
| 1H, 1H, 9H-hexadecafluoro-1-monomethacrylate | 65-85             |
| 1H, 1H, 5H-octafluoro-1-pentanoacrylate      | 14-30             |
| Acrylic acid                                 | 1-5               |
| Triallycyanurate                             | 0.3-1             |
| Azo-bisisobutyronitrile                      | 0.1-1             |

20

18. A binder composition comprising the following constituents:

| Constituents                                 | Percent by weight |
|----------------------------------------------|-------------------|
| 1H, 1H, 9H-hexadecafluoro-1-monomethacrylate | 65-79             |
| 1H, 1H, 5H-octafluoro-1-pentanoacrylate      | 17-30             |
| Acrylonitrile                                | 1.5-5             |
| Triallycyanurate                             | 0.3-1             |
| Azo-bisisobutyronitrile                      | 0.1-0.5           |

30

19. A binder composition comprising the following constituents:

| Constituents                                 | Percent by weight |
|----------------------------------------------|-------------------|
| 1H, 1H, 9H-hexadecafluoro-1-monomethacrylate | 53-60             |
| 1H, 1H, 5H-octafluoro-1-pentanoacrylate      | 20-24             |
| Dinitropropylacrylate                        | 5-20              |
| Azo-bisisobutyronitrile                      | 0.1-0.3           |
| Triallycyanurate                             | 0.3-1             |

45

\* \* \* \* \*

55

60

65

70

75